

April 18, 1967

C. E. RANSLEY

3,314,876

METHOD FOR MANUFACTURING SOLID CURRENT CONDUCTING ELEMENTS

Original Filed Dec. 16, 1960

3 Sheets-Sheet 1

FIG. 1



FIG. 2



INVENTOR  
CHARLES ERIC RANSLEY

BY *James E. Toomey*  
ATTORNEY

April 18, 1967

C. E. RANSLEY

3,314,876

METHOD FOR MANUFACTURING SOLID CURRENT CONDUCTING ELEMENTS

Original Filed Dec. 16, 1960

3 Sheets-Sheet 2

Fig. 3



Fig. 4



Fig. 5



INVENTOR

CHARLES ERIC RANSLEY

BY

*James E. Rooney*

ATTORNEY

April 18, 1967

C. E. RANSLEY

3,314,876

METHOD FOR MANUFACTURING SOLID CURRENT CONDUCTING ELEMENTS

Original Filed Dec. 16, 1960

3 Sheets-Sheet 3



FIG. 6



FIG. 7



FIG. 8



FIG. 9

INVENTOR  
CHARLES ERIC RANSLEY

BY

*James E. Ransley*

ATTORNEY

# United States Patent Office

3,314,876

Patented Apr. 18, 1967

1

3,314,876

## METHOD FOR MANUFACTURING SOLID CURRENT CONDUCTING ELEMENTS

Charles Eric Ransley, Chesham Bois, England, assignor to The British Aluminium Company Limited, London, England, a company of Great Britain  
Original application Dec. 16, 1960, Ser. No. 76,265. Divided and this application Jan. 27, 1966, Ser. No. 523,300

Claims priority, application Great Britain, Nov. 28, 1960, 40,853/60  
4 Claims. (Cl. 204—291)

This application is a division of Ser. No. 76,265, filed Dec. 16, 1960, now abandoned, which application Ser. No. 76,265 is a continuation-in-part of application Ser. No. 764,725 filed Oct. 1, 1958, and now U.S. Patent 3,215,615, issued Nov. 2, 1965.

This invention relates to improvements in solid current conducting elements for use in the production of aluminum and methods of manufacturing such elements and is particularly concerned with such elements intended to extend into the interior of an electrolytic reduction cell for the production of aluminum or a three-layer refining cell, such an element constituting the cathode of a reduction cell or taking part in the supply of electrolyzing current to a body of molten metal either in a reduction cell or in a refining cell. Such elements, whether used as cathodes or current supply leads, all come into contact with molten aluminum at some part of their surface.

In the specifications of British Patents Nos. 784,695, 784,696, and 802,471 there are described various such current conducting elements which have the common feature that they are largely composed of at least one of the materials titanium carbide and zirconium carbide. In the specification of British Patent No. 802,905 it is stated that such a current conducting element may also be made having at least part of its surface intended to be exposed to the interior of the cell largely composed of at least one of the materials in the group consisting of the borides of titanium, zirconium, tantalum and niobium and particular reference is made to the excellent properties of titanium diboride  $TiB_2$ . In particular, it has a much lower electrical resistivity than titanium carbide, is more resistant to oxidation in the temperature range 300° to 800° C., and has a lower solubility in molten aluminum at the temperatures found in aluminum producing electrolytic cells, i.e., 950° to 1000° C. This last property is extremely important in the commercial exploitation of such current conducting elements since the life of the elements is ultimately determined by the rate at which the material thereof dissolves in the aluminum in the electrolytic cell.

Although the borides of the elements referred to are significantly superior to the carbides thereof for the purposes in view they were, until hitherto, more expensive to produce than the carbides. In the specification of British Patent No. 826,635 I have described and claimed a current conducting element for use in an electrolytic cell for the production of aluminum, which element is intended to come into contact with molten aluminum during its use, characterized in that at least that portion of the element which is to contact the aluminum is largely composed of a mixture of titanium carbide and titanium boride. Such a mixture has various advantages which could not be anticipated from a study of their properties determined separately and special reference is made to the surprising reduction in the solubility of titanium carbide in aluminum at high temperatures (e.g., at 970° C.) which can be achieved by small percentage additions of titanium boride, additions of 5 to 25% by weight of titanium boride being particularly mentioned.

It was found that the oxygen content of the carbides of

2

titanium, zirconium, tantalum and niobium is an important factor in the solubility of the compounds in molten aluminum. In my co-pending application Ser. No. 764,725 filed Oct. 1, 1958, now Patent No. 3,215,615, I have described and claimed a solid current conducting element for use in an electrolytic cell for the production or purification of aluminum and adapted to have at least a part thereof exposed to a body of molten aluminum or aluminum alloy within the cell wherein at least said part of said element consists essentially of at least one of the materials in the group consisting of the carbides of titanium, zirconium, tantalum and niobium and the oxygen content of said materials is less than 1% by weight.

The expressions "largely composed of" and "consisting essentially of" as used hereinafter in the specification and the claims, mean that the current conducting element, or at least the portion thereof which is adapted to be in contact with molten aluminum, made of at least one of the carbides and/or borides referred to above does not contain other substances in amounts sufficient to materially affect the desirable characteristics of the current conducting element, although other substances may be present in minor amounts which do not materially affect such desirable characteristics, for example, small proportions of carbon, nitrogen, or iron. In order for the element to "consist essentially" or be "largely composed" of at least one of the carbides and/or borides as described above the oxygen impurity content should be limited as hereafter prescribed. Further, these expressions are used to denote that the current conducting element, or at least the portion thereof adapted to contact molten aluminum during use, desirably, but not essentially contains at least 90% by weight of at least one of the carbides and/or borides referred to.

Although the borides of the chemical elements referred to are markedly superior to the carbides thereof for the purposes in view, my experiments on the manufacture of solid current conducting elements largely composed of titanium diboride and titanium diboride-titanium carbide mixtures, which are technically of great importance, have shown that unexpected difficulties can occur in the control of the quality of such elements. Thus in my experimental work, a proportion of the elements were found to be quite unsuitable for use in reduction or refining cells because they failed prematurely under cell operating conditions, this proportion being sufficiently high to reflect adversely on the possibility of manufacturing such elements commercially. This failure was associated with a clearly defined tendency to crack and disintegrate within the cell. Micrographic examination of elements or bars after service showed that in poor materials exhibiting this deficiency, a characteristic intergranular penetration of aluminum had occurred which eventually led to complete disruption of the structure. This effect was absent in materials which behaved in a satisfactory manner, even when such materials were sufficiently porous to allow some aluminum to infiltrate into the interior in use, because even under these conditions the aluminum remained localized in the pores, and did not spread between the grains. These effects could be produced in molten pure aluminum as well as under electrolytic conditions. This quality factor could in fact be characterized in terms of the so-called "dihedral angle" (as defined, for example, in the paper by C. S. Smith in the Transactions of the American Institute of Mining and Metallurgy 1948, volume 175, page 15) made by the aluminum phase at its conjunction with a grain boundary, in the structure. When this angle was about 60° or more, no penetration between the grains occurred and the material was found suitable for cell applications; when, on the other hand, this angle was less than this (e.g. 20—30°) disintegration of the structure inevitably occurred and the material was quite unsuitable for cell use.

In order to indicate how good and poor materials may be distinguished by appropriate chemical analysis and to give an understanding of the complex constitution of these materials, it is desirable to indicate the processes by which they may be manufactured.

Continually improving techniques have materially reduced the cost of preparing titanium diboride,  $TiB_2$ , and the various processes are available for its preparation. The most important ones are considered to be the carbothermic process, electrolytic separation and direct reaction between the chemical elements. The carbothermic process may involve any one of several reactions, one of which involves reacting  $TiO_2$  (anatase or rutile),  $B_2O_3$  and carbon according to the following equation:



An alternative reaction is one in which the boron is supplied in the form of boron carbide (nominally  $B_4C$ ):



Elemental boron may also be used in accordance with the equation:



Boron, however, is difficult to produce in a pure enough form for the purposes in view, and this is not at present regarded as an economic route.

An alternative reaction which may be employed is as follows:



Reactions (2), (3) and (4) are obviously variants of the basic reaction given in Equation 1.

In addition to carbothermic processes, the most direct way of preparing the borides is by reaction of the elements:



In this case again, however, the main objection is the difficulty of preparing elemental boron of the necessary purity at an economical price.

Various electrolytic processes have also been proposed for the preparation of the borides. These do not normally offer any technical or economic advantage over the carbothermic or direct reaction processes; however, even for this product, the considerations to be detailed below are still applicable.

It is extremely difficult in practice to achieve an exact stoichiometric balance in a carbothermic, or any other reaction for the preparation of  $TiB_2$ , as is implicit, for example, in Equation 2 above. There are technical difficulties, for example, in providing exactly the correct amounts of boron and carbon; this is because somewhat variable losses can occur during the reaction, accidental contamination may take place, and the atmosphere in which the process is carried out may also have an effect on the composition of the final product. A further possibility is that the reaction may not have proceeded as far to completion as the make-up of the reaction mass would allow under appropriate conditions.

The product obtained from such reactions will thus contain, to a greater or lesser degree, components other than the simple compound  $TiB_2$ . Thus, if the reaction mixture contains an inadequate supply of boron or boron compounds to combine with all the titanium present, and carbon is present over and above that required for the elimination of oxygen, the product will contain an appreciable amount of titanium carbide,  $TiC$ . In fact, it is probably not inaccurate to regard  $TiC$  as a primary product of the carbothermic preparation; it tends to be unstable in the presence of boron, however, in conformity with the reaction:



Similarly, if the mixture is deficient in both boron and carbon, the product will be contaminated with oxygen in some form or other. The other possible variations in

composition which can occur do not need detailed description, but it will be evident that the final product may possibly contain, for example, excess boron carbide and free (or uncombined) carbon. In addition, a number of contaminating elements may be present which are derived from the raw materials or from the atmospheres used; these may include, for example, relatively small quantities of nitrogen, iron, calcium, silicon and aluminum.

The final product of such carbothermic or other processes is normally in the form of a relatively fine powder, which has been subjected to milling or other operations to render it suitable for further fabrication.

The solid conducting elements referred to are produced by either cold pressing followed by sintering, or by hot-pressing this powder, an appropriate protective atmosphere being used in both these operations. For example, it may be hot pressed in a graphite die, in a protective atmosphere of hydrogen, and at temperatures of the order of 1800-2100° C. It will be understood that the chemical composition of the final element thus obtained will be determined not only by the exact composition of the powder used, but also by the conditions under which the element is manufactured from it. Precise control of the final composition of the element is essential, however, if the latter is to have a useful economic life in an electrolytic cell.

We have found, unexpectedly, that the elements exhibiting poor behavior do so because of the presence therein of a relatively small percentage of oxygen combined in a certain manner, and it has further been found that the permissible content of oxygen of this type is related to the so-called soluble, or combined, carbon content of the material. The discovery of this interrelation between the oxygen and carbon contents of such elements has enabled us for the first time to control their composition in such a way that no cracking or disintegration occurs in service.

According to the present invention, a solid conducting element for use in the electrolytic production or purification of aluminum has at least a portion consisting essentially of at least one of the materials titanium diboride and titanium carbide and has an oxygen impurity content, defined as that oxygen present in the element in chemical combination with titanium which is less than 0.1% by weight when the combined (or acid-soluble) carbon content is less than 0.4% by weight, and is less than  $(0.1 + 0.04 \times n)\%$  by weight when the combined carbon content is  $n\%$  by weight, and the value of  $n$  is greater than 0.4.

Preferably the element contains titanium carbide in the proportion of not more than 40% by weight and desirably not less than 2% by weight.

From the analytical point of view, the proportion of acid-soluble carbon present defines the combined carbon content, which is normally ascribable to the formula  $TiC$ . In analysis, this figure is usually derived by carrying out a determination of the total carbon content of the material, and a separate determination of the acid-insoluble or filtrable carbon residue remaining after the mass of the sample is dissolved in an appropriate acid or acid mixture; this latter figure thus includes graphitic and elemental carbon, and also carbon in the residual boron carbide. The acid-soluble carbon is then obtained from the difference between these two figures, and this is the value of carbon content which is specified above to which the tolerable oxygen content is related.

The oxygen content of the final element may conveniently be determined by the well-known vacuum fusion method, in which a sample is reduced in a high temperature bath of molten iron or platinum contained in a graphite crucible, and the consequent evolution of carbon oxide measured. The sample may, for example, comprise a relatively massive chip or cut section of the element. If the element is powdered in order to obtain

a representative sample and for convenience in general analysis, spurious oxygen will be introduced in the form of titanium oxide and boric oxide ( $B_2O_3$ ) on the surface of the particles, and also as absorbed water; appropriate correction must therefore be made in order to obtain the oxygen content which is significant in the present context. Methods are available for this; thus the  $B_2O_3$  content can be determined by aqueous extraction of the powder, and the water content can be deduced from the hydrogen evolved in the vacuum-fusion measurement.

It is clearly essential to be able to assess the quality of element which will be obtained by hot-pressing or otherwise consolidating a given batch of powder into the said element. Since it is desired that the oxygen content, as defined above, of the final product shall be as low as possible, a minimum requirement is that the proportion of reducing agents present shall be adequate to eliminate this oxygen from the powder.

Both carbon and boron are capable of functioning as reducing agents. For reasons which are explained in more detail below, it has been found preferable to adjust the composition of the charge in the carbothermic reaction so that the powder for pressing and also the final element contains an appreciable percentage, e.g., 0.2% or more, of acid-soluble carbon, or about 1% or more of  $TiC$ . Oxygen will be evolved from a powder of this type during hot-pressing or sintering by reaction with the free, or other available, carbon with a loss of carbon monoxide from the system. Oxygen present as titanium oxide (e.g.,  $TiO$ ) is able to react as follows:



and the carbon required render these conditions such that the weight ratio  $O/C$  is not greater than  $\frac{16}{12} = 0.66$ . However, if boron is available in the powder either as unreacted boron or boron carbide, or even as  $B_2O_3$ , further carbon is made available by reaction of this boron with  $TiC$  to form  $TiB_2$  and releasing carbon as expressed in Equation 6. Under these conditions the basic carbon requirement is then given by

$$O < \frac{16}{12} = 1.33$$

the carbon available from reaction 6 in percent by weight is 0.56 times the percentage of boron present in the powder other than as  $TiB_2$ . A requirement for the control of quality of the powder is thus:

$$\frac{\text{Total O to be reduced}}{\text{Total C available for reduction}} =$$

Total O by vacuum fusion

Free C + 0.56 × B content < 1.33 other than  $TiB_2$

If a mixture is used in which an excess of boron is intended, the  $TiC$  content of the carbothermic powder tends to be low by virtue of the reaction shown in Equation 6, i.e., the carbon is displaced by boron. The undesirable oxygen content can then be reduced by reaction with boron; the product obtained,  $B_2O_3$ , is not harmful to quality and since it is quite volatile at high temperatures, some is lost from the element during the hot-pressing or sintering operation. There are some very inconvenient consequences of this type of compositional control, however, which render it undesirable. Thus, a high  $B_2O_3$  content tends to cause sticking of the powder in the die during hot-pressing so that a high degree of compaction cannot be obtained without adopting special precautions. In addition, it is found that the electrical resistivity of the final element is higher than in materials with an appreciable  $TiC$  content and that the oxidation resistance is also poorer.

Accordingly, the present invention also provides a powder for use in the manufacture of a solid current conducting element for use in an electrolytic cell for the production of aluminum which powder consists essentially of at least one of the materials titanium diboride

and titanium carbide and wherein the ratio of total oxygen present in the powder in percent by weight to the total carbon available in the powder for reduction in percent by weight is less than 1.33.

5 It is preferred that the powder should contain boron in an amount less than that required by the stoichiometric ratio for the titanium present and carbon in addition to that required for reduction in an amount sufficient to compensate for this deficiency of boron.

10 The invention also provides as a further feature, a method of producing a solid current conducting element for use in an electrolytic cell for the production of aluminum which comprises hot-pressing or cold-pressing and subsequently sintering a powder according to either of 15 the two immediately preceding paragraphs.

15 It is preferred to hot-press the powder to a density such that the porosity does not exceed 10% by volume although a greater porosity can be tolerated provided it does not exceed 20% by volume. Good results have 20 been achieved with a powder having a particle size which averages  $6\mu$  with a deviation of  $2.5\mu$  but higher particle sizes can be tolerated and smaller particle sizes are preferred.

25 As mentioned above, commercial production of titanium diboride (e.g., using reaction 2 above) automatically introduces a number of contaminating elements of which the principal ones are iron, carbon, nitrogen and oxygen. Traces of other elements such as calcium, silicon and aluminum are also present, usually totalling not more

30 than 0.5% by weight and these, in such small proportions, do not appear to be significant. Carbon and oxygen usually derive from the basic material and nitrogen is principally derived from air contamination and adsorption in the carbon black employed as one of the

35 starting materials. Iron is derived from two main sources (a) original impurity in the starting material and (b) pick-up in grinding and ball-milling operations. Generally speaking, the iron content should be less than 0.5% by weight although a higher content can be tolerated.

40 The nitrogen content should be less than 0.3% by weight for a percentage by weight of combined carbon of up to 0.4%, not more than 0.6% by weight at 10% combined carbon (corresponding to 50% by weight of titanium carbide) and not more than 1% by weight at 20% combined carbon (corresponding to 100% by weight of titanium carbide) although a higher content can be tolerated.

45 It is preferred that the free carbon content of the final element should not exceed 0.8% by weight.

50 Six examples of the manufacture of solid current conducting elements will now be given:

#### Example I

55 4200 g. of ball-milled titanium diboride powder prepared by a carbothermic process was taken for fabrication. This powder had a mean cumulative particle size as determined by sedimentation in water, of approximately  $6\mu$  with a standard deviation of approximately  $2.5\mu$ . It had the following chemical analysis:

| (Powder M.18)             | Weight percent | Equivalent compounds | Weight percent |
|---------------------------|----------------|----------------------|----------------|
| Acid-soluble boron.....   | 29.21          | $TiB_2$ .....        | 93.9           |
| Titanium.....             | 66.4           | .....                | .....          |
| Acid-insoluble boron..... | 0.28           | .....                | .....          |
| "Free" carbon.....        | 0.70           | .....                | .....          |
| Soluble carbon.....       | 0.88           | $TiC$ .....          | 4.40           |
| Iron.....                 | 0.22           | .....                | .....          |
| Nitrogen.....             | 0.05           | .....                | .....          |
| Total oxygen.....         | 1.11           | .....                | .....          |
|                           |                |                      | 98.80          |

In the above analysis, and in those given subsequently, the so-called "acid-soluble boron" includes a small portion of water-soluble boron, which may be present as

$B_2O_3$  or hydrolysable borides of impurity elements, or both.

The powder was pressed in a 2 in. diameter graphite die in an atmosphere of hydrogen, with an applied pressure which was increased in appropriate steps from  $\frac{1}{4}$  5 ton/sq. in. to a final value of 1 ton/sq. in., the temperature being raised from cold to 2000-2050° C. in about 3½-4 hours.

The rod obtained, which was approximately 20 in. long, had the following properties which could be determined 10 by non-destructive testing:

Density (overall) (89% theoretical) 4.02  
Electrical resistivity, microhm. cm. 19.4

The chemical analysis of the material, carried out on a 15 sample of the rod crushed to -90 mesh B.S.S., was as follows:

| (Rod B.100/414)           | Weight percent | Equivalent compounds        | Weight Percent | 20 |
|---------------------------|----------------|-----------------------------|----------------|----|
| Acid-soluble boron.....   | 29.38          | TiB <sub>2</sub> .....      | 94.3           |    |
| Titanium.....             | 68.6           | .....                       |                |    |
| Acid-insoluble boron..... | 0.17           | .....                       |                |    |
| "Free" carbon.....        | 0.29           | .....                       |                |    |
| Soluble carbon.....       | 0.76           | TiC.....                    | 3.80           | 25 |
| Iron.....                 | 0.26           | .....                       |                |    |
| Nitrogen.....             | 0.07           | .....                       |                |    |
| Total oxygen.....         | 0.51           | Oxygen as "titanium oxide." | 0.07           |    |
|                           | 100.04         |                             |                | 30 |

The "titanium oxide" content was deduced by subtracting the spurious oxygen (associated with water vapor and surface oxidation produced by the powdering process) from the total oxygen. A check figure obtained by measurement of the total oxygen content of a large fragment or chip of bar (which required only a very small correction for spurious oxygen) gave 0.11% oxygen at titanium oxide.

This rod was provided with an aluminum lead at one end in the manner specified in British Patent No. 825,443, and was used as a top-entering lead in an experimental reduction cell as described in my U.S. application Ser. No. 660,994, filed May 23, 1957, now Patent No. 3,028,324. It carried current for a period of 122 days without any cracking or serious deterioration within the molten flux and metal zone of the cell, and with very little solution (a reduction in diameter of only 0.008 in.).

This was thus representative of a final fabricated material suitable for cell application.

### Example II

4200 g. of titanium boride powder of similar physical characteristics to that specified in Example I were taken; this batch had the following analysis:

| (Powder 211/2)            | Weight percent | Equivalent compounds   | Weight Percent | 55 |
|---------------------------|----------------|------------------------|----------------|----|
| Acid-soluble boron.....   | 28.54          | TiB <sub>2</sub> ..... | 91.7           |    |
| Titanium.....             | 67.1           | .....                  |                |    |
| Acid-insoluble boron..... | 0.07           | .....                  |                |    |
| "Free" carbon.....        | 0.20           | .....                  |                |    |
| Soluble carbon.....       | 0.79           | TiC.....               | 3.95           |    |
| Iron.....                 | 0.78           | .....                  |                |    |
| Nitrogen.....             | 0.15           | .....                  |                |    |
| Total oxygen.....         | 1.33           | .....                  |                |    |
|                           | 98.94          |                        |                |    |

The powder was hot-pressed on a similar schedule to Example I, and a 2 in. diameter rod approximately 20 in. long obtained with the following properties:

Density (overall) (91% theoretical) 4.11  
Electrical resistivity, microhm. cm. 13.6

The chemical analysis of the crushed rod was determined as follows:

| (Rod B. 100/235)          | Weight percent | Equivalent compounds        | Weight percent |
|---------------------------|----------------|-----------------------------|----------------|
| Acid-soluble boron.....   | 28.78          | TiB <sub>2</sub> .....      | 92.5           |
| Titanium.....             | 67.20          | .....                       |                |
| Acid-insoluble boron..... | 0.07           | .....                       |                |
| "Free" carbon.....        | 0.02           | .....                       |                |
| Soluble carbon.....       | 0.60           | TiC.....                    | 3.00           |
| Iron.....                 | 0.92           | .....                       |                |
| Nitrogen.....             | 0.20           | Oxygen as "titanium oxide." | 0.63           |
| Total oxygen.....         | 0.94           | .....                       |                |
|                           | 98.73          |                             |                |

The "titanium oxide" was deduced as in Example I.

The rod was provided with an aluminum lead as previously described, and was used as a top-entering lead in a reduction cell in the same manner as in Example I. It failed to carry current after a period of immersion of less than 2 days, and when removed for examination showed multiple cracking, mostly of a radial character, which rendered it useless.

Material of this nature was thus clearly quite unsuitable for cell applications.

### Example III

2250 g. of titanium boride powder of similar physical characteristics to that specified in Examples I and II were taken; this batch had the following analysis:

| (Powder 278)              | Weight percent | Equivalent compounds   | Weight percent |
|---------------------------|----------------|------------------------|----------------|
| Acid-soluble boron.....   | 29.32          | TiB <sub>2</sub> ..... | 94.2           |
| Titanium.....             | 67.5           | .....                  |                |
| Acid-insoluble boron..... | 0.06           | .....                  |                |
| "Free" carbon.....        | 0.48           | .....                  |                |
| Soluble carbon.....       | 1.00           | TiC.....               | 5.0            |
| Iron.....                 | 0.60           | .....                  |                |
| Nitrogen.....             | 0.06           | .....                  |                |
| Total oxygen.....         | 0.62           | .....                  |                |
|                           | 99.64          |                        |                |

This powder was hot-pressed on a similar schedule to that described for Example I, except that because of the smaller weight of charge it was pressed in a different die assembly, and the time taken to reach the maximum temperature of about 2050° C. was only 1½ hours.

The rod obtained was approximately 10 in. long and had the following properties:

Density (overall) (89% theoretical) 4.03  
Electrical resistivity, microhm. cm. 18.0  
Transverse rupture strength, tons/sq. in. 15.4

The chemical analysis of the crushed rod was determined as follows:

| (Rod B.100/297)           | Weight percent | Equivalent compounds        | Weight percent |
|---------------------------|----------------|-----------------------------|----------------|
| Acid-soluble boron.....   | 29.35          | TiB <sub>2</sub> .....      | 94.2           |
| Titanium.....             | 68.03          | .....                       |                |
| Acid-insoluble boron..... | 0.05           | .....                       |                |
| "Free" carbon.....        | 0.09           | .....                       |                |
| Soluble carbon.....       | 0.97           | TiC.....                    | 4.85           |
| Iron.....                 | 0.73           | .....                       |                |
| Nitrogen.....             | 0.03           | Oxygen as "titanium oxide." | 0.08           |
| Total oxygen.....         | 0.43           | .....                       |                |
|                           | 99.68          |                             |                |

The "titanium oxide" content was deduced as in Example I.

Half of this bar was subjected to an immersion test in a reduction cell. For this test it was placed in the pool (or "pad") of molten aluminum at the bottom of a reduction cell operating under normal conditions; after immersion for 129 days, it was recovered for examination and found to be quite sound and free from cracks. The

diameter had decreased by 0.11 in. during this immersion. The rather higher rate of solution than that quoted in Example I arose from the conditions of test. In the test described in Example I, sufficient  $TiB_2$  rods were inserted into the molten metal to produce saturated solution conditions, whereas in the immersion tests the metal was not fully saturated.

Material of this composition was thus judged suitable for cell applications.

*Example IV*

2250 g. of titanium boride powder of similar physical characteristics to that specified in Examples I, II and III were taken; this batch had the following analysis:

| (Powder 217/8)            | Weight percent | Equivalent compounds | Weight percent |
|---------------------------|----------------|----------------------|----------------|
| Acid-soluble boron.....   | 28.72          | $TiB_2$ .....        | 92.3           |
| Titanium.....             | 67.7           |                      |                |
| Acid-insoluble boron..... | 0.04           |                      |                |
| "Free" carbon.....        | 0.26           |                      |                |
| Soluble carbon.....       | 0.67           | $TiC$ .....          | 3.35           |
| Iron.....                 | 0.74           |                      |                |
| Nitrogen.....             | 0.15           |                      |                |
| Total oxygen.....         | 1.27           |                      |                |
|                           | 99.55          |                      |                |

This powder was hot-pressed on a similar schedule to that described for Example III.

The rod obtained was approximately 10 in. long and had the following properties:

Density (overall), (90.5% theoretical) ..... 4.10  
Electrical resistivity, microhm. cm. ..... 14.2  
Transverse rupture strength, tons/sq. in. ..... 5.7

The chemical analysis of the crushed rod was determined as follows:

| (Rod B.100/241)           | Weight percent | Equivalent compounds             | Weight percent |
|---------------------------|----------------|----------------------------------|----------------|
| Acid-soluble boron.....   | 29.01          | $TiB_2$ .....                    | 93.2           |
| Titanium.....             | 68.2           |                                  |                |
| Acid-insoluble boron..... | 0.04           |                                  |                |
| "Free" carbon.....        | 0.04           |                                  |                |
| Soluble carbon.....       | 0.44           | $TiC$ .....                      | 2.20           |
| Iron.....                 | 0.74           |                                  |                |
| Nitrogen.....             | 0.14           | Oxygen as "titanium oxide."..... | 0.59           |
| Total oxygen.....         | 0.79           |                                  |                |
|                           | 99.40          |                                  |                |

The "titanium oxide" content was deduced as in Examples I, II and III.

Half of this bar was subjected to an immersion test in a reduction cell in the same manner as described in Example III. This was recovered after 6 days and was found to be badly cracked and virtually disintegrated.

Material of this composition was thus clearly unsuitable for cell applications.

*Example V*

Titanium diboride powder was ball-milled with 10% by weight of titanium carbide powder, and the final milled material was analyzed as follows:

| (Powder 365)              | Weight percent | Equivalent compounds | Weight percent |
|---------------------------|----------------|----------------------|----------------|
| Acid-soluble boron.....   | 26.49          | $TiB_2$ .....        | 85.1           |
| Titanium.....             | 67.4           |                      |                |
| Acid-insoluble boron..... | 0.44           |                      |                |
| "Free" carbon.....        | 0.84           |                      |                |
| Soluble carbon.....       | 2.56           | $TiC$ .....          | 12.8           |
| Iron.....                 | 0.13           |                      |                |
| Nitrogen.....             | 0.06           |                      |                |
| Total oxygen.....         | 1.20           |                      |                |
|                           | 99.12          |                      |                |

200 g. of the powder were hot-pressed on a similar schedule to that described in Examples III and IV.

The rod obtained was approximately 10 in. long and had the following properties:

Density (overall) (95.2% theoretical) ..... 4.36  
5 Electrical resistivity, microhm. cm. ..... 16.6  
Tranverse rupture strength, tons/sq. in. ..... 14.6

The chemical analysis of the crushed rod was determined as follows:

| 10 (Rod B. 90/8)          | Weight percent | Equivalent compounds             | Weight percent |
|---------------------------|----------------|----------------------------------|----------------|
| Acid-soluble boron.....   | 27.36          | $TiB_2$ .....                    | 87.8           |
| Titanium.....             | 68.8           |                                  |                |
| Acid-insoluble boron..... | 0.08           |                                  |                |
| "Free" carbon.....        | 0.48           |                                  |                |
| Soluble carbon.....       | 2.37           | $TiC$ .....                      | 11.85          |
| Iron.....                 | 0.15           |                                  |                |
| Nitrogen.....             | 0.07           | Oxygen as "titanium oxide."..... | 0.17           |
| Total oxygen.....         | 0.42           |                                  |                |
|                           | 99.73          |                                  |                |

Half of this rod was subjected to an immersion test in a reduction cell in the same manner as previously described. It was recovered after 92 days and was found to be quite sound and free from cracks; the diameter had decreased by 0.08 in.

This material was thus judged suitable for cell applications.

*Example VI*

30 Titanium diboride powder was ball-milled with 10% by weight of titanium carbide powder and the final milled material was analyzed as follows:

| 35 (Powder 363)           | Weight percent | Equivalent compounds | Weight percent |
|---------------------------|----------------|----------------------|----------------|
| Acid-soluble boron.....   | 26.28          | $TiB_2$ .....        | 84.5           |
| Titanium.....             | 68.8           |                      |                |
| Acid-insoluble boron..... | 0.08           |                      |                |
| "Free" carbon.....        | 0.25           |                      |                |
| Soluble carbon.....       | 2.43           | $TiC$ .....          | 12.10          |
| Iron.....                 | 0.55           |                      |                |
| Nitrogen.....             | 0.14           |                      |                |
| Total oxygen.....         | 0.85           |                      |                |
|                           | 99.38          |                      |                |

45 2000 g. of the powder was hot-pressed on a similar schedule to that described in Examples III, IV and V.

The rod obtained was approximately 10 in. long and had the following properties:

Density (overall) (97.3% theoretical) ..... 4.46  
50 Electrical resistivity, microhm. cm. ..... 14.6  
Transverse rupture strength, tons/sq. in. ..... 17.7

The chemical analysis of the crushed rod was determined as follows:

| 55 (Rod B.90/1)           | Weight percent | Equivalent compounds             | Weight percent |
|---------------------------|----------------|----------------------------------|----------------|
| Acid-soluble boron.....   | 26.36          | $TiB_2$ .....                    | 84.7           |
| Titanium.....             | 69.5           |                                  |                |
| Acid-insoluble boron..... | 0.04           |                                  |                |
| "Free" carbon.....        | 0.03           |                                  |                |
| Soluble carbon.....       | 2.35           | $TiC$ .....                      | 11.75          |
| Iron.....                 | 0.57           |                                  |                |
| Nitrogen.....             | 0.14           | Oxygen as "titanium oxide."..... | 0.36           |
| Total oxygen.....         | 0.54           |                                  |                |
|                           | 99.53          |                                  |                |

65 Half of this rod was subjected to an immersion test in a reduction cell in the same manner as previously described. It was recovered after 21 days and was found to be badly cracked.

Material of this composition was thus clearly unsuitable for cell applications.

The oxygen content of a solid current conducting element produced as described above, other than that due to  $B_2O_3$  or oxygen absorbed during powdering of the

element to analyze it, is considered to be mainly present in the form of oxygen associated with the metal, e.g., titanium oxide and it will be observed from the above examples that the elements produced in accordance with Examples I, III and V, all of which were suitable for the purposes in view, conform to the requirement that the combined or acid soluble carbon content of the element in percent by weight is less than 0.1% when the combined carbon content is no greater than 0.4% and is less than  $(0.1+0.04 \times n)$  percent where  $n$  is said combined carbon content and is greater than 0.4%. This relationship is due to the fact that when the combined carbon is greater than 0.4%, the oxygen, in the form of titanium oxide  $TiO_2$ , can exist in solid solution in the carbide, which appears as a second phase.

An analysis of the powders used in and of the final elements or rods produced by the above examples is set out in the following table. In this table, total carbon available for reduction is calculated on the basis total carbon-free carbon + 0.56 (acid-insol B + water-sol B).

TABLE I

| Example | Powder Analysis, percent by weight |               |              |                                 |         | Ratio, O/C | Rod Analysis, percent by weight |                 | Quality |  |
|---------|------------------------------------|---------------|--------------|---------------------------------|---------|------------|---------------------------------|-----------------|---------|--|
|         | "Free C"                           | Acid insol. B | Water sol. B | Total C available for reduction | Total O |            | O as "titanium oxide"           | Residual Free C |         |  |
|         |                                    |               |              |                                 |         |            |                                 |                 |         |  |
| I       | 0.70                               | 0.23          | 0.15         | 0.91                            | 1.11    | 1.2        | 0.07                            | 0.29            | Good.   |  |
| II      | 0.20                               | 0.07          | 0.47         | 0.50                            | 1.33    | 2.65       | 0.63                            | 0.02            | Bad.    |  |
| III     | 0.48                               | 0.06          | 0.07         | 0.54                            | 0.62    | 1.15       | 0.08                            | 0.90            | Good.   |  |
| IV      | 0.26                               | 0.04          | 0.43         | 0.52                            | 1.27    | 2.4        | 0.59                            | 0.04            | Bad.    |  |
| V       | 0.84                               | 0.44          | 0.12         | 1.15                            | 1.20    | 1.05       | 0.17                            | 0.48            | Good.   |  |
| VI      | 0.25                               | 0.08          | 0.16         | 0.38                            | 0.85    | 2.3        | 0.36                            | 0.03            | Bad.    |  |

It will be observed from this table that the powders from which a good element was produced conform to the requirement that the ratio of total oxygen to total carbon available for reduction should be less than 1.33.

It is apparent from our investigations that in a solid current conducting element consisting essentially of at least one of the materials titanium diboride and titanium carbide, the quantity of oxygen present in the form of the oxide of the metal is a determining factor. It would appear that when this quantity of oxygen is higher than a predetermined value which is a function of the combined or acid-soluble carbon content of the element, the element is attacked by molten aluminum which penetrates the element and causes it to crack and/or disintegrate.

It will be apparent from the above disclosure that an unsuitable powder can, under appropriate conditions, be made suitable by increasing the free carbon content thereof and/or by increasing the boron content thereof (other than in the form of the boride of the metal). As higher oxygen contents can be tolerated with increasing proportions of the carbide of the metal, a bad powder can sometimes be changed to a good powder by increasing the amount of titanium carbide present. This is not a disadvantage as I have found that the very pure borides present difficulties in pressing to the final form as they do not densify readily and there is a tendency for sticking to occur in the graphite die. It is therefore preferred that a solid current conducting element consisting of at least one of the materials titanium diboride and titanium carbide should contain from 2 to 40% by weight of titanium diboride or titanium carbide and desirably not less than 10% by weight.

Some examples of electrolytic cells embodying solid current conducting elements according to the invention will now be briefly described with reference to the accompanying drawings in which:

FIGS. 1 to 7 are sectional views of reduction cells, and

FIGS. 8 and 9 are sectional views of three-layer refining cells.

In the example illustrated in FIG. 1 pairs of opposed solid cathodes 1 of plate form and consisting essentially of at least one of the materials titanium diboride and titanium carbide are supported by walls 2 at a small angle to the vertical one on each side of an appropriately shaped anode 3. The right-hand wall 2 is omitted in this figure. The cathodes 1 are immersed in molten electrolyte 4 containing dissolved alumina and extend at their lower end into the pool of molten aluminum 5 which forms on the floor of the cell. Current leads 6 which also consist essentially of at least one of the materials titanium diboride and titanium carbide extend through the wall of the cell in the pool of molten aluminum 5 and are connected at their outer ends to the negative pole of the D.C. supply. The pool of molten aluminum 5, in this example, forms part of the current supply system and also acts as a cathode. The usual crust of solidified flux which forms over the cell is indicated at 7.

The arrangement illustrated in FIG. 2 is very similar to that illustrated in FIG. 1 and like references are used to denote like parts. In this case, the current leads 6

are omitted and replaced by extensions 1a of the cathodes which extend through the crust 7 for connection to the negative pole of the D.C. supply. These extensions 40 are provided with protective sleeves 8 where they extend through the crust 7, these sleeves being of aluminum or a refractory material.

The arrangement illustrated in FIG. 3 is similar to that illustrated in FIG. 1 but in this case, the solid cathodes 1 are omitted together with their supporting walls 2 and the pool of molten aluminum 5 constitutes the sole cathode.

The arrangement illustrated in FIG. 4 is similar to that shown in FIG. 3 but in this case the current leads 6 do not extend through the wall of the cell but extend into the pool of molten aluminum 5 through the crust 7 at the side of the cell and are provided with a protective sleeve 8. It is preferred, however, that the current leads 6 should be arranged as indicated in FIG. 5 substantially centrally of the cell between anodes 3 as this arrangement leaves the sides of the cell free for replenishing the cell and the crust 7 is thinner at the center than at the sides. Additionally this arrangement lends itself to an arrangement of bus-bars (not shown) whereby magnetic effects can be reduced to a minimum.

FIG. 6 shows an arrangement in which the current leads 6 extend through the floor of the cell.

FIG. 7 shows how an existing cell may be modified to include current leads 6 according to the invention, these leads being embedded in the carbon floor 9 of the cell 65 which is connected to the negative pole of the D.C. supply by iron bars 10 embedded therein. The current leads extend up into the pool of molten aluminum 5 through any sludge layer which may be formed on the floor of the cell and so avoid the power loss which such a layer otherwise introduces.

FIG. 8 shows a three-layer refining cell having the usual lower layer 11 of molten aluminum alloy, intermediate layer 12 of electrolyte and upper layer 13 of purified aluminum. The lower layer 11 is connected to the positive 75 pole of a D.C. supply by current leads 6a extending

through the wall of the cell and the upper layer 13 is connected to the negative pole of the D.C. supply by current leads 6b extending through the wall of the cell, the current leads 6a and 6b consisting essentially of at least one of the materials titanium diboride and titanium carbide.

In a three-layer cell illustrated in FIG. 9 the current leads 6b are shown extending into the upper layer 13 from the top of the cell and are provided with protective sheaths 8.

Although the foregoing disclosure relates to titanium carbide and titanium boride and mixtures thereof, it is to be understood that the carbides and borides of zirconium, tantalum and niobium are to be included. In connection with these metals, however, due to the different atomic weights, the percentage weight limitation on the oxygen content defined in relation to titanium carbide and titanium boride and mixtures thereof together with the percentage by weight of the combined acid-soluble carbon content is to be multiplied by a factor equal to the ratio of the atomic weight of titanium to the atomic weight of zirconium, tantalum or niobium as the case may be. Where mixtures of the carbides and/or borides of two or more of the metals are concerned, this factor will be modified in accordance with the relative proportions of the metals present.

It will be obvious that various modifications and alterations may be made in this invention without departing from the spirit and scope thereof and it is not to be taken as limited except by the appended claims, wherein what is claimed is:

1. A method of producing a current conducting element having high resistance to failure under aluminum producing electrolytic cell operating conditions, said method comprising:

5

10

15

25

30

35

pressing powder consisting essentially of a mixture of titanium diboride and titanium carbide, said powder also containing small proportions of oxygen and free carbon; and

maintaining the present weight ratio of total oxygen present in the powder to the total carbon available in the powder for reduction of oxygen at a value of less than 1.33.

2. A method according to claim 1 wherein the total available carbon is comprised of free carbon.

3. A method according to claim 1 wherein the total available carbon percentage is comprised of the percent by weight free carbon plus .56 times the percent by weight of the acid insoluble and water soluble boron materials present in the powder.

4. A method of producing a current conducting element for use in electrolytic cells for the production of aluminum having reduced tendency to fail under cell operating conditions comprising sintering at least one powder material having an oxygen and carbon content of a mixture of titanium diboride and titanium carbide, said powder material having a ratio in percent by weight of total oxygen to total carbon available in the powder material for reduction of oxygen, of less than 1.33.

#### References Cited by the Examiner

##### UNITED STATES PATENTS

|           |         |               |         |
|-----------|---------|---------------|---------|
| 2,813,069 | 11/1957 | Raynes et al. | 204-294 |
| 2,915,442 | 12/1959 | Lewis         | 204-243 |
| 3,028,324 | 4/1962  | Ransley       | 204-279 |

JOHN H. MACK, Primary Examiner.

D. R. JORDAN, Assistant Examiner.